

July 1, 1952

P. N. MURPHY

2,601,863

METHOD OF CLEANING HOT-DIP TIN-PLATE

Filed April 6, 1948



Inventor:  
PAUL N. MURPHY,  
by: Donald G. Dalton  
his Attorney.

## UNITED STATES PATENT OFFICE

2,601,863

## METHOD OF CLEANING HOT-DIP TIN-PLATE

Paul N. Murphy, Hobart, Ind., assignor to United States Steel Company, a corporation of New Jersey

Application April 6, 1948, Serial No. 19,303

3 Claims. (Cl. 134—15)

1

This invention relates to the manufacture of tin-plate and, in particular, to an improved finishing treatment thereof, i. e., the processing subsequent to the coating with tin, whereby discoloration or the formation of surface film is avoided.

Prime tin-plate should exhibit a bright silvery appearance and be free from visible surface films or discoloration, but complete freedom from discoloration is difficult to achieve under the present manufacturing practice. Two types of discoloration are frequently encountered. The first is the development of a straw-yellow color on the sheet when it is heated incident to lithographing or other processes during fabrication. The second is the appearance of a similar or even deeper color on the sheets before shipment from the manufacturer to the customer. It has been observed that the higher the temperature of the palm-oil bath through which the tinned sheets emerge from the molten tin in the ordinary hot-dip tinning process, the greater the tendency to discoloration. If the palm oil is kept below the temperature which causes discoloration, however, the result is the formation of heavy list edges and beads of tin on the sheets. While such defects were not considered very serious in the past, they have now become so because of the increasingly high standards of quality established and maintained by tin-plate users.

The finishing of tin-plate as now conducted includes a washing of the sheets to remove a portion of the palm oil adhering thereto and a branning operation for drying and polishing them. All the oil is not removed by the washing, however, because it has been generally accepted that a solution strong enough to do so would etch the sheets. As a result, the amount of oil remaining cannot be precisely controlled and is frequently more or less than is considered desirable by the user. The branning operation is objectionable, furthermore, because of the dust created thereby in the tin house and further because the bran contaminates the surface of the material and results in "eye-holing" or discontinuous adherence of the lacquer film applied to the sheets before fabrication of certain articles, such as packing cans. Many sheets are cobbled or otherwise damaged in the branning machine, furthermore, and have to be scrapped.

It is accordingly the primary object of my invention to provide a method of finishing tin-plate whereby the product is free from discoloration as well as heavy list edges and beads.

2

A further object is to simplify the finishing process and reduce the cost thereof. A still further object is to eliminate the branning operation entirely. Another object is to achieve complete removal of oil from the sheets during the washing.

In a preferred practice of the invention, I deliver sheets of hot-dip tin-plate, as they emerge from the palm oil bath floating on the molten tin in the tin-pot, without cooling and while the oil adhering thereto is still fluid, directly into a wash tank. After immersion in a solution of soda ash contained therein, they are conveyed to a second wash tank containing a similar but less concentrated solution and are then spray-rinsed with hot water. The first washing solution is strong enough to remove substantially all palm oil from the sheets. As a final operation, therefore, I apply to the sheets just the precise amount of oil desired by the trade.

A complete understanding of the invention may be obtained from the following detailed description and explanation which refer to the accompanying drawings illustrating apparatus for carrying out the present preferred practice. In the drawings:

Figures 1 and 2 together constitute a central vertical section through a line of apparatus for subjecting tinned sheets to the finishing treatment of my invention.

Referring in detail to the drawings, the apparatus there shown includes a tin-pot 10 of conventional construction, a first wash tank 11, a second wash tank 12, spray pipes 13, an oiler 14 and delivery pinch rolls 15. The tin-pot 10 is of known construction and the showing thereof is largely diagrammatic since no detailed description is necessary. It has a plurality of exit rolls 16 therein. Deflecting rolls 16a above the tin-pot progressively bend the sheets emerging successively therefrom for delivery laterally of the pot. A guide chute 17 extends downwardly from a point adjacent the deflector rolls and directs each sheet between a pair of entry or feed-in rolls 18 journaled on the near side of the wash tank 11. Additional pairs of traction rolls 19 and 20 convey the sheet through the washing solution contained in the tank 11. The sheet is then passed between two pairs of wiping rolls 21 which remove excess washing solution by squeegee action, and discharged onto a roller table 22.

The sheet is then delivered to entry rolls 23 of the second wash tank 12 and is carried through a washing solution contained therein by addi-

tional traction rolls 24 and 25. The last of these delivers the sheet to two pairs of wiping rolls 26 which remove excess solution therefrom and deliver the sheet to a roller table 27. As the sheet passes over the table, it is subjected to a hot-water rinse by spray jets from pipes 13. A tank 28 is provided below the table for collecting the rinse water flowing from the sheet.

The oiler 14 through which the sheet then passes comprises a pair of pinch rolls 29 which feed the sheet forward onto a roller table 30. Oil is supplied to the rolls 29 by a stack of rolls 31, the upper one of which engages the bottom pinch roll. The bottom roll 31 rides on a wick 32 immersed in palm oil contained in a reservoir 33. The rolls 31 are provided with wiper blades 34 for controlling the amount of oil transferred thereby.

After passing through the oiler and being delivered by the pinch rolls thereof onto the table 30, the sheet is engaged by pinch rolls 15 and delivered thereby to a piler (not shown).

The apparatus preferred for carrying out my improved method having been described in detail, it remains to explain further the successive operations performed thereby upon the tinned sheet. The operation of the tin-pot is similar to prior practice except that I maintain the temperature of the palm-oil bath floating on the molten tin at a temperature between 460° and 480° F. The upper limit is controlled so that the tin coating will be solidified by the time the sheet reaches the last set of exit rolls 16. This facilitates handling of the material during subsequent processing. Moreover, it obviously eliminates heavy list edges and beads of tin which would adhere to the sheet if the oil were maintained at a lower temperature. With the oil at the temperature stated, it remains highly fluid as the sheet bends over and falls down onto the guide 17. This is advantageous from the standpoint of complete removal of the oil from the sheet in the two-stage cleaning afforded by the tanks 11 and 12. To insure entry of the sheets into the first wash tank before substantial cooling of the sheet and stiffening of the oil thereon, the first wash tank is placed as close as possible to the tin-pot and the cooling conveyor, usually incorporated in a tinning line, is omitted or made as short as possible.

The first wash tank 11 contains an aqueous solution of from 0.5% to 1.5% of soda ash or anhydrous sodium carbonate. The solution is heated to a temperature of from 180° to 200° by any suitable means. The conveying rolls in the wash tank are driven and preferably the two rolls of each pair are driven at slightly different speeds, thereby producing a rubbing action on the sheet. The speed of the rolls is such as to cause the sheet to be immersed in the solution for from 5 to 10 seconds. The solution in the first wash tank, by reason of its concentration and temperature, is effective to remove most of the oil adhering to the sheet as a result of its passage through the palm-oil bath floating on the molten tin, on emerging from the tin-pot. The wiping rolls 21 remove washing solution adhering to the sheet and deliver it to the roller table 22 from which it enters the second wash tank 12. This tank contains an aqueous solution of from 0.10% to 0.25% of soda ash or anhydrous sodium carbonate and is maintained at approximately the same temperature as the solution in the first wash tank. The rolls in the tank 12 are driven in the same manner as those of tank 11. As the

sheet passes through the solution in tank 11, the last trace of adherent palm oil is removed. Excess washing solution is removed from the sheet as it traverses the rolls 36 and it is then thoroughly rinsed by the spray jets of hot water (180°-200° F.) from pipes 13 as it passes along the table 27.

The final operation of my improved method is the application to the sheet of a predetermined amount of palm oil as it passes through the rolls 29 of oiler 14. It will be evident that, in the interval between the passage of successive sheets, the rolls 31 will transfer a film of oil from the wick to the rolls 29. This film is applied to the sheet as it passes between the last-mentioned rolls. As a result, the sheets emerging onto the roller table 30 have a predetermined coating of oil on both sides thereof. The amount of oil transferred from the wick to the pinch rolls 29 and applied thereby to the sheet is controlled by adjusting the wiper blades 34 engaging the transfer roll 31 and varying the speed of the latter. The finished sheets, coated with palm oil, are delivered by the pinch rolls 15 to a piler and, after piling, are ready to be stored or shipped.

It will be apparent from the foregoing that the method of my invention is characterized by numerous advantages. In the first place, the sheets produced thereby are characterized by unusual freedom from discoloration despite the fact that the palm-oil bath in the tin-pot is maintained at a higher temperature than has heretofore been thought feasible. As a matter of fact, the material produced by my method is entirely free from discoloration when shipped and does not develop this defect when lithographed under normal conditions. The tendency of tin-plate to discolor is graded on a numerical scale from zero to ten, the latter indicating very bad discoloration. My method makes possible the production of tin-plate possessing stain resistance of grades 1 and 2. This compares with the production of grades 3 and 4 by the conventional method of finishing tin-plate.

A further advantage is that the luster and reflectivity of tin-plate processed by my method are greater than that of the product resulting from the prior practice while no spangling is produced. My method, furthermore, eliminates the branning treatment altogether and thus does away with difficulties resulting from "eye-holding" as well as the objectionable contamination of the air in the vicinity of the processing apparatus by bran dust. Finally, the percentage of prime sheets produced is substantially increased as a result of the elimination of the branner in which cobbling or other damage to the sheets frequently occurs. As a result, the invention makes possible a reduction in maintenance and production costs.

Although I have illustrated and described but a preferred practice of the invention, it will be understood that changes in the procedure disclosed may be made without departing from the spirit of the invention or the scope of the appended claims.

I claim:

1. In a method of finishing hot-dip tin-plate, the steps including delivering sheets as they emerge from the palm oil floating on the molten tin in a tin-pot, before substantial cooling of the sheets, directly into a hot soda-ash solution having a concentration between .5% and 1.5%, then passing the sheets through a second hot soda-ash solution having a concentration between .10%

and .25%, thereby removing substantially all the oil adhering to the sheets on leaving the tin-pot.

2. The method defined by claim 1 characterized by maintaining said solutions at a temperature between 180° and 200° F.

3. The method defined by claim 1 characterized by maintaining said palm oil at a temperature between 460° and 480° F.

P. N. MURPHY.

#### REFERENCES CITED

The following references are of record in the file of this patent:

#### UNITED STATES PATENTS

| Number    | Name  | Date           |
|-----------|-------|----------------|
| 2,141,382 | Ferm  | Dec. 27, 1938  |
| 2,357,970 | Rath  | Sept. 12, 1944 |
| 2,359,088 | Croft | Sept. 26, 1944 |